

# United States Patent [19]

Titov et al.

[11] 3,753,717

[45] Aug. 21, 1973

[54] **PHOTOGRAPHIC MATERIAL**

[76] Inventors: Alexei Alexeevich Titov, ulitsa Gatvalda 18a, KV. 65; Jury Vasilievich Smirnov, poselok Moskvorechie 48, KV. 48; Jury Shabsaevich Mashkovsky, Zubovsky bulvar 16/20, KV. 2, all of Moscow; Ernest Dmitrievich Tamitsky, Pushkinsky raion, stantsia Mamontovka, ulitsa Oktyabrskaya 22, Moskovskaya oblast; Vladimir Nikitovich Chursin, ulitsa Gari baldi 7, KV. 5, Moscow; Ljudmila Leonidovna Antonova, stantsia Podlipki, proezd Makarevko, 8, KV. 18, Moskovskaya oblast; Tamara Stepanovna Selitskaya, Krasny Stroitel, 2 Kvartal, 1, KV. 31, Moscow, all of U.S.S.R.

[22] Filed: Feb. 3, 1972

[21] Appl. No.: 223,338

[52] U.S. Cl..... 96/88, 96/92, 96/94,  
96/114.6

[51] Int. Cl..... G03c 1/00

[58] Field of Search..... 96/88, 114.6, 94,  
96/92

[56] **References Cited**

UNITED STATES PATENTS

3,658,534 4/1972 Ishitani et al. .... 96/88 R

Primary Examiner—Norman G. Torchin  
Assistant Examiner—Richard L. Schilling  
Attorney—Eric H. Waters et al.

[57] **ABSTRACT**

A photographic material, comprising a support with a mixture applied thereto, said mixture comprising an organic dye such as methylene blue or thionine blue, a water-soluble salt of silver, gold, platinum or palladium and disodium salt of ethylenediaminetetraacetic acid or triethanolamine. The content of said components in said mixture is the following (g per m<sup>2</sup> of the support surface area):

|                                                                         |                                        |
|-------------------------------------------------------------------------|----------------------------------------|
| organic dye                                                             | 5·10 <sup>-3</sup> -5·10 <sup>-2</sup> |
| water-soluble salt of silver,<br>gold, platinum or palladium            | 1·10 <sup>-3</sup> -5·10 <sup>-2</sup> |
| disodium salt of ethylenediamine tetraacetic acid or<br>triethanolamine | 2.5-20                                 |

Said mixture may also comprise gelatine or polyvinyl alcohol in an amount of 2-50 g per m<sup>2</sup> of the support surface area.

The photographic material according to the invention exhibits light sensitivity both in ultraviolet and visible regions of the spectrum. This permits to use this photographic material to produce negative and positive images when taking photographs and reproducing coloured objects.

3 Claims, No Drawings

## PHOTOGRAPHIC MATERIAL

The present invention relates to a photographic material which is light-sensitive both in ultraviolet and visible regions of the spectrum. Such a material may be used in conventional and scientific photography, cinematography, in making microfilms and in documents duplication, as well as in printing.

Known in the art is a photographic material, comprising a support with a mixture of a light-sensitive material such as a trivalent iron salt, and a salt of a noble metal, such as palladium, applied thereto.

This prior-art photographic material exhibited very low light sensitivity and was sensitive only to the ultraviolet region of the spectrum. For this reason, commercial application of this photographic material was very limited, since it must be used with special ultraviolet light sources, very long exposure and highly expensive quartz optical systems. Furthermore, a restricted range of spectral sensitivity makes this photographic material absolutely unsuitable for taking photographs (that is, this photographic material cannot be used as negative material).

It is an object of the present invention to provide a photographic material which is light-sensitive both in ultraviolet and visible regions of the spectrum.

In accordance with this and other objects, the invention consists in the provision of a photographic material, comprising a support with a mixture applied thereto, said mixture comprising an organic dye, such as methylene blue or thionine blue, a water-soluble salt of silver, gold, platinum or palladium and disodium salt of ethylenediamine-tetraacetic acid or triethanolamine, said mixture containing the following quantities of said components (g per m<sup>2</sup> of the support surface area):

|                                                                     |                                         |
|---------------------------------------------------------------------|-----------------------------------------|
| organic dye                                                         | 5·10 <sup>-3</sup> - 5·10 <sup>-2</sup> |
| water-soluble salt of silver, gold, platinum or palladium           | 1·10 <sup>-3</sup> - 5·10 <sup>-2</sup> |
| disodium salt of ethylenediaminetetraacetic acid or triethanolamine | 2.5 - 20                                |

The photographic material according to the invention is sensitive both in ultraviolet and visible regions of the spectrum, whereby it may be used to obtain negative and positive images in reproducing colour objects.

In the material according to the invention a visible image is built up by a conventional method of physical development of latent image centers consisting in reducing ions of a cheap metal, such as copper, mercury, nickel on said centers. This results in a considerable reduction of the consumption of an expensive metal, such as silver, which takes place when silver halide photographic materials are used. In order to produce half-tone photographic images having fine grains, it is desirable to use a photographic material comprising 2-50 g per m<sup>2</sup> of the support surface area of gelatine or polyvinyl alcohol.

In order to increase the quantum yield of photochemical reaction, and hence to increase light sensitivity of the photographic material according to the invention, a water-soluble salt of bivalent copper, trivalent iron or tetravalent tin in an amount of 1·10<sup>-2</sup> - 5·10<sup>-1</sup> g per m<sup>2</sup> of the support surface area is introduced into the material.

The photographic material according to the invention is prepared in the following manner.

Aqueous solutions of each of the above-said components having a predetermined concentration are prepared and then mixed in a predetermined ratio in darkness or when exposed to the light of an incandescent lamp screened with a blue filter.

When preparing the photographic material to be used in making line copies of documents, a paper support is impregnated with the mixture of the components thus prepared (without introducing gelatine and polyvinyl alcohol).

When preparing the photographic material to be used for high-grade half-tone images, the mixture of components thus prepared (including also gelatine or polyvinyl alcohol) is applied to a support (paper, triacetyl cellulose, glass) to produce a uniform layer using 1 l of an aqueous solution per m<sup>2</sup> of the support surface.

Impregnated paper support or light-sensitive layer applied to the support is dried at 20°-60°C.

Exposure of the photographic material thus prepared is made in daylight or in the light of an incandescent lamp (without a filter or through an orange or red filter, if necessary) during 0.5 to 5 minutes with the illumination of the lightsensitive layer of 100-500 luxes.

Upon the exposure the material is soaked for 10-15 minutes in water or, which is better, in a slightly acidic solution in order to prevent reversible (dark) reaction and eliminate the unreacted substances interfering with the development. After the soaking all operations with the exposed material are performed in any light.

The exposed material is developed with a physical developer. Known physical developers may be used, such as mercury, copper, nickel developer and the like. The development is performed at room temperature for 0.1 to 1 hour.

Upon the physical development, the photographic material is washed with running water during 10-20 minutes and is then dried in air or in drying apparatus at 40°-80°C.

The photographic material according to the invention may be used in making line copies of documents, negative and positive half-tone pictures, in taking photographs and in making reproductions of coloured objects.

Better understanding of the present invention may be had from the following examples illustrating the preparation and application of the photographic material according to the invention.

## EXAMPLE 1

An aqueous solution of the following composition (g/l) was prepared:

|                                                   |                    |
|---------------------------------------------------|--------------------|
| methylene blue                                    | 5·10 <sup>-2</sup> |
| disodium salt of ethylenediamine-tetraacetic acid | 20                 |
| silver nitrate                                    | 5·10 <sup>-2</sup> |

The pH of the solution was of 4.5 - 5.5.

In order to prepare this solution, aqueous solutions of each of the above-mentioned components were first separately prepared in any light. Then these solutions were mixed in the light of an incandescent lamp of 25 W screened with a blue filter, which was placed at a distance of 1 m from the working zone.

The resulting light-sensitive solution was used for impregnating a paper support by applying 400 ml of the solution per m<sup>2</sup> of the support surface. The impregnation was effected at room temperature and in the

above-mentioned non-actinic light. Then the support was dried in air for 1 hour.

The resulting photographic material comprised a support of pale blue colour impregnated with the light-sensitive composition. This material was sensitive substantially to yellow and red regions of the spectrum.

The photographic material thus prepared was used to produce positive copies from negative line pictures (texts, documents drawings). The photographic material was exposed during 5 minutes through a negative by a contact method in the light of an incandescent lamp of 500 W placed at a distance of 1 m.

Upon the exposure, the material was soaked in water for 10-15 minutes. This operation was performed in the above-said non-actinic light. After the soaking, the material exhibited no light sensitivity, and its further treatment (physical development, washing and drying) was done in any light.

Visible image was obtained by means of physical development of the latent image using mercury physical developer. In order to prepare this developer, two aqueous solutions of the following composition (g/l) were first prepared:

|                             |      |
|-----------------------------|------|
| Solution I                  |      |
| Mercury nitrate             | 8.35 |
| Potassium bromide           | 8.0  |
| Crystalline sodium sulphite | 120  |
| Solution II                 |      |
| Metol                       | 20   |
| Crystalline sodium sulphite | 40   |

The solutions (I) and (II) were mixed in a ratio 5:1 respectively before the development. The pH of the developer was of 7.8-8.1. The development was effected at 25°C for 15 minutes and a consumption of the developer of 1 l per 2 m<sup>2</sup> of the surface of the exposed photographic material.

Upon the development, the photographic material was washed with running water for 15 minutes and dried in air during 1 hour.

The resulting line image had the following characteristics:

|                            |      |
|----------------------------|------|
| maximum density, $D_{max}$ | 1.4  |
| minimum density, $D_{min}$ | 0.3  |
| fog density, $D_0$         | 0.07 |

The image was built up with contrasting black lines.

## EXAMPLE 2

An aqueous solution of the following composition (g/l) was prepared:

|                 |                     |
|-----------------|---------------------|
| methylene blue  | $5 \cdot 10^{-2}$   |
| triethanolamine | 20                  |
| silver nitrate  | $1 \cdot 10^{-2}$   |
| copper sulphate | $2.5 \cdot 10^{-2}$ |

The pH of the solution was of 10-11.

The preparation of the light-sensitive solution, its application to a paper support, exposure and treatment of the exposed photographic material were performed similarly to Example 1.

The resulting line positive image exhibited the same characteristics as in Example 1.

## EXAMPLE 3

An aqueous solution of the following composition (g/l) was prepared:

|          |    |
|----------|----|
| gelatine | 50 |
|----------|----|

|                                                   |                   |
|---------------------------------------------------|-------------------|
| methylene blue                                    | $8 \cdot 10^{-3}$ |
| disodium salt of ethylenediamine-tetraacetic acid | 9.3               |
| silver nitrate                                    | $3 \cdot 10^{-3}$ |

5 The pH of the solution was 4.5-5.5.

The solution was prepared according to Example 1. Then the solution was applied at 40°C and in non-actinic light, to produce a uniform layer, to a support of cellulose triacetate, using 1 l of the solution per m<sup>2</sup> of the support surface. Upon the application of the light-sensitive solution to the support it was cooled at 3°-5°C for 1 minute and then dried at 40°C during 30 minutes.

When viewed in a passing light, the resulting photographic material was transparent (there was no turbidity) due to homogeneous structure of the layer.

The photographic material was used to produce half-tone negative images. In doing this, the photographic material was exposed for 1 minute in the light of an incandescent lamp of 500 W placed at a distance of 1 m.

Upon the exposure, the photographic material was soaked as described in Example 1, after which it exhibited no light sensitivity. Further treatment of the material (physical development, washing and drying) was performed in any light.

A latent image was developed by means of a mercury physical developer similar to that described in Example 1. The development was effected at 25°C for 30 minutes.

Upon the development, the photographic material was washed in running water during 20 minutes and dried in air for one hour.

The resulting half-tone image exhibited the following characteristics:

|                            |      |
|----------------------------|------|
| maximum density, $D_{max}$ | 1.8  |
| minimum density, $D_{min}$ | 0.1  |
| fog density, $D_0$         | 0.05 |

The photographic image was built up with progressive change of density from  $D_{max}$  to  $D_{min}$  and was of dark grey colour.

## EXAMPLE 4

45 An aqueous solution of the following composition (g/l) was prepared:

|                                                   |                     |
|---------------------------------------------------|---------------------|
| gelatine                                          | 50                  |
| methylene blue                                    | $1 \cdot 10^{-2}$   |
| disodium salt of ethylenediamine-tetraacetic acid | 9                   |
| ferrous sulphate (oxy-salt)                       | $4 \cdot 10^{-2}$   |
| silver nitrate                                    | $1.7 \cdot 10^{-2}$ |

55 The pH of the solution was of 4.5-5.5.

The solution was prepared as described in Example 1. Then the solution was applied to a paper support at 40°C and in non-actinic light to produce a uniform layer using 1 l of the solution per m<sup>2</sup> of the support surface. Upon the application of the light-sensitive solution to the support it was cooled at 3°-5°C for 1 minute and dried at 40°C during 30 minutes.

The resulting photographic material was used to produce half-tone positive images. In doing this, the photographic material was exposed during 40 seconds through a negative by a contact method in the light of an incandescent lamp of 500 W placed at a distance of 1 m.

Upon the exposure, the material was soaked in a 0.1 percent aqueous solution of sulphuric acid, after which the material exhibited no light sensitivity.

Visible image was obtained by means of the development of the latent image using a physical developer. In order to prepare this developer, two aqueous solutions were first prepared. Solution I had the following composition:

|                             |     |
|-----------------------------|-----|
| crystalline copper sulphate | 7   |
| potassium tartrate          | 22  |
| sodium hydroxide            | 4.5 |

Solution II was a 1 percent aqueous solution of formaldehyde. Before the development, solutions I and II were mixed in a volumetric ratio of 1:1. The pH of the developer was 10-11. The development was performed at 25°C for 10 minutes using 1 l of the developer per m<sup>2</sup> of the exposed photographic material.

Upon the development, the photographic material was washed with running water for 20 minutes and dried in air during one hour.

The resulting half-tone image exhibited the following characteristics:

|                                   |      |
|-----------------------------------|------|
| maximum density, D <sub>max</sub> | 1.0  |
| minimum density, D <sub>min</sub> | 0.09 |
| fog density, D <sub>f</sub>       | 0.08 |

The photographic image was built up with progressive change of density from D<sub>max</sub> to D<sub>min</sub> and was of brown colour.

#### EXAMPLE 5

An aqueous solution of the following composition (g/l) was prepared:

|                 |                    |
|-----------------|--------------------|
| gelatine        | 30                 |
| methylene blue  | 8·10 <sup>-3</sup> |
| triethanolamine | 5                  |
| copper sulphate | 1·10 <sup>-2</sup> |
| silver sulphate | 5·10 <sup>-2</sup> |

The pH of the solution was 10-11.

The solution was prepared similarly to that of Example 1. Then the solution was applied to a glass support at 40°C and in non-actinic light to produce a uniform layer using 1 l of the solution per m<sup>2</sup> of the support surface. Upon the application of the light-sensitive solution to the support, it was cooled at 3°-5°C for 1 minute and dried at 40°C during 30 minutes.

The resulting photographic material was used to produce half-tone positive images, the conditions of exposure and further treatment of the photographic material being similar to those described in Example 1.

The resulting half-tone image exhibited the following characteristics:

|                                   |      |
|-----------------------------------|------|
| maximum density, D <sub>max</sub> | 1.3  |
| minimum density, D <sub>min</sub> | 0.08 |
| fog density, D <sub>f</sub>       | 0.05 |

The photographic image was built up with progressive change of density from D<sub>max</sub> to D<sub>min</sub> and was of black colour.

#### EXAMPLE 6

An aqueous solution of the following composition (g/l) was prepared:

|                |                    |
|----------------|--------------------|
| gelatine       | 50                 |
| methylene blue | 9·10 <sup>-3</sup> |

|                                                    |                    |
|----------------------------------------------------|--------------------|
| disodium salt of ethylene-diamine-tetraacetic acid | 20                 |
| tetravalent tin nitrate                            | 5·10 <sup>-1</sup> |
| tetravalent gold chloride                          | 4·10 <sup>-3</sup> |

5 The pH of the solution was of 4.5 - 5.5.

The preparation of the light-sensitive solution, its application to a paper support and the treatment of the material upon the exposure were performed as described in Example 4.

10 The resulting half-tone image exhibited the following characteristics:

|                                   |      |
|-----------------------------------|------|
| maximum density, D <sub>max</sub> | 1.2  |
| minimum density, D <sub>min</sub> | 0.1  |
| fog density, D <sub>f</sub>       | 0.09 |

15 The photographic image was built up with progressive change of density from D<sub>max</sub> to D<sub>min</sub> and was of brown colour.

#### EXAMPLE 7

An aqueous solution of the following composition (g/l) was prepared:

|                                                    |                    |
|----------------------------------------------------|--------------------|
| polyvinyl alcohol                                  | 50                 |
| methylene blue                                     | 8·10 <sup>-3</sup> |
| disodium salt of ethylene-diamine-tetraacetic acid | 9.3                |
| tetravalent tin chloride                           | 4·10 <sup>-2</sup> |
| tetravalent platinum chloride                      | 1·10 <sup>-3</sup> |

30 The pH of the solution was of 4.5 - 5.5.

The preparation of the light-sensitive solution and its application to a paper support were performed as described in Example 4.

35 The resulting photographic material was used to produce half-tone positive images. In doing this, the photographic material was exposed during 1 minute through a negative by a contact method in the light of an incandescent lamp of 500 W placed at a distance of 1 m.

40 The exposed material was then soaked in water for 10-15 minutes, after which the material exhibited no light sensitivity.

45 Visible image was obtained by means of physical development, using a nickel physical developer. In order to prepare this developer two aqueous solutions were first prepared. Solution I had the following composition (g/l):

|                   |      |
|-------------------|------|
| nickel sulphate   | 28   |
| potassium citrate | 32.4 |

50 Solution II comprised an aqueous solution of sodium hypophosphite with a concentration of 240 g/l. Before the development solutions I and II were mixed in a volumetric ratio of 4:1 respectively. The pH of the developer was 10-11.

55 Upon the exposure, the photographic material was developed during 15 minutes at 80°C using 1 l of the developer per 5 m<sup>2</sup> of the photographic material surface area.

Upon the development, the photographic material was washed in running water for 25 minutes and dried in air for one hour.

The resulting half-tone image exhibited the following characteristics:

|                                   |      |
|-----------------------------------|------|
| maximum density, D <sub>max</sub> | 1.8  |
| minimum density, D <sub>min</sub> | 0.1  |
| fog density, D <sub>f</sub>       | 0.09 |

The photographic image was built up with progressive change of density from  $D_{max}$  to  $D_{min}$  and was of black colour.

## EXAMPLE 8

An aqueous solution of the following composition (g/l) was prepared:

|                                                  |                   |
|--------------------------------------------------|-------------------|
| polyvinyl alcohol                                | 20                |
| methylene blue                                   | $5 \cdot 10^{-3}$ |
| disodium salt of ethylenediaminetetraacetic acid | 2.5               |
| copper chloride                                  | $3 \cdot 10^{-2}$ |
| palladium sulphate                               | $1 \cdot 10^{-3}$ |

The pH of the solution was 4.5 – 5.5.

The preparation of the light sensitive solution, its application to a paper support, exposure and treatment of the exposed material were performed as described in Example 7.

The resulting half-tone positive image was built up with progressive change of density from  $D_{max}$  to  $D_{min}$  and was of dark colour.

## EXAMPLE 9

An aqueous solution of the following composition (g/l) was prepared:

|                                                  |                   |
|--------------------------------------------------|-------------------|
| polyvinyl alcohol                                | 25                |
| methylene blue                                   | $5 \cdot 10^{-2}$ |
| disodium salt of ethylenediaminetetraacetic acid | 10                |
| copper sulphate                                  | $5 \cdot 10^{-2}$ |
| tetravalent platinum chloride                    | $1 \cdot 10^{-3}$ |

The pH of the solution was 4.5 – 5.5.

The preparation of the light sensitive solution was performed as described in Example 1. Then the solution was applied to a glass support at 40°C and in non-actinic light to produce a uniform layer using 1 l of the solution per  $m^2$  of the support. Upon the application of the light-sensitive solution to the support, it was cooled at 3°–5°C for 1 minute and dried at 40°C during 30 minutes.

The resulting photographic material was used to produce half-tone negative images. In doing this, the material was exposed during one minute in the light of an incandescent lamp of 500 W placed at a distance of 1 m.

Upon the exposure, the material was soaked in water, developed in a physical developer, washed in running water and dried as described in Example 7.

The resulting negative photographic image exhibited the following characteristics:

|                            |      |
|----------------------------|------|
| maximum density, $D_{max}$ | 2.5  |
| minimum density, $D_{min}$ | 0.1  |
| fog density, $D_f$         | 0.07 |

The photographic image was built up with progres-

sive change of density from  $D_{max}$  to  $D_{min}$  and was of black colour.

## EXAMPLE 10

5 An aqueous solution of the following composition (g/l) was prepared:

|                                                  |                   |
|--------------------------------------------------|-------------------|
| gelatine                                         | 2                 |
| thionine blue                                    | $5 \cdot 10^{-2}$ |
| disodium salt of ethylenediaminetetraacetic acid | 20                |
| tetraacetic acid                                 | $4 \cdot 10^{-2}$ |
| ferrous sulphate (oxy-salt)                      | $2 \cdot 10^{-2}$ |
| silver nitrate                                   |                   |

The pH of the solution was 4.5 – 5.5.

The preparation of the light-sensitive solution, its application to a paper support, exposure and treatment of the exposed photographic material were performed according to Example 1.

The resulting line positive image exhibited the following characteristics:

|                            |     |
|----------------------------|-----|
| maximum density, $D_{max}$ | 1.3 |
| minimum density, $D_{min}$ | 0.4 |
| fog density, $D_f$         | 0.1 |

25 The photographic image was built up with contrasting lines having black colour.

We claim:

1. A photographic material, comprising a support with a mixture applied thereto, said mixture comprising an organic dye, selected from the group consisting of methylene blue and thionine blue, a water-soluble salt of a metal selected from the group consisting of silver, gold, platinum and palladium, and an amino-compound selected from the group consisting of disodium salt of ethylenediaminetetraacetic acid and triethanolamine, the content of said components in said mixture being the following (g per  $m^2$  of the support surface area):

|                                                |                                     |
|------------------------------------------------|-------------------------------------|
| organic dye                                    | $5 \cdot 10^{-3} - 5 \cdot 10^{-2}$ |
| water-soluble salt of one of said noble metals | $1 \cdot 10^{-3} - 5 \cdot 10^{-2}$ |
| amino-compound                                 | 2.5 – 20                            |

2. A photographic material according to claim 1, wherein said mixture also comprises a binder selected from the group consisting of gelatine and polyvinyl alcohol in an amount of 2–50 g per  $m^2$  of a support surface area.

3. A photographic material according to claim 1, wherein said mixture further comprises a water-soluble salt of a metal selected from the group consisting of bivalent copper, trivalent iron and tetravalent tin in an amount of  $1 \cdot 10^{-2} - 5 \cdot 10^{-1}$  g per  $m^2$  of the support surface area.

\* \* \* \* \*